

## UNITED STATES PATENT OFFICE

2,172,041

## PICKLING SOLUTION

Stephen F. Urban, Chicago, Ill.

No Drawing. Application October 7, 1937,  
Serial No. 167,859

1 Claim. (CL. 148-8)

This invention relates to pickling solutions and, particularly, to such a solution for pickling chromium alloy steels such as chrome steels and chrome-nickel steels.

5 In the course of manufacture of chromium steel alloy or chromium-nickel steel alloy articles, sheets, etc., a scale is formed on the surface thereof. This scale has to be removed for various reasons before such articles can be used commercially. As is generally known, it is the usual practice to remove the scale by immersing the articles in a pickling solution after the final annealing operation.

10 It is an object of this invention to provide a pickling solution which will remove this scale from such metals without pitting, corroding or otherwise damaging the surface thereof.

15 It has been found that annealed chrome steels and alloys thereof, with or without nickel, and 20 with or without such additions as titanium, columbium or molybdenum, can be successfully pickled to remove the scale in a pickling solution containing hydrofluoric acid mixed with an oxidizing reagent such as chromic acid, potassium chromate, potassium dichromate or potassium permanganate, and with or without sulphuric acid. Such a pickling solution has been found especially satisfactory for use in connection with 25 chrome steels or alloys thereof containing more than 12 per cent of chromium, with or without nickel, and with or without such additions as titanium, columbium or molybdenum. These 30 solutions may be used either hot or cold, and their composition may be varied to satisfy the individual case for which they are adapted to be used.

35 It has been found that a satisfactory pickling solution for most cases contains from 5 to 20 per

cent by volume of a suitable oxidizing agent, such as chromic acid, potassium chromate, potassium dichromate or potassium permanganate, mixed with from  $\frac{1}{2}$  of 1 per cent to 10 per cent by volume of hydrofluoric acid and with sulphuric acid in amounts up to 10 per cent by volume, the remaining percentage of the solution, of course, being water. For example, if chromic acid is used as the oxidizing reagent, the pickling solution would then contain from 10 to 20 per cent by 5 volume of chromic acid, and from 1 to 10 per cent by volume of hydrofluoric acid and up to 10 per cent by volume of sulphuric acid mixed with water. The percentages of the amount of acid used, of course, depends upon the type of scale on the 10 article to be pickled. It will be understood, of course, that the acid concentration of the solution continuously decreases during the pickling operation, thereby decreasing the relative initial amounts of the ingredients of the acids used; 15 therefore the concentration of the solution has to be increased by replenishing acid from time to time.

20 Such a solution will effectively and efficiently remove the scale in a very short period of time and yet will not attack the surface of the metal under the scale.

## 1-claim:

25 A pickling solution for removing scale from chromium alloy steels, such as chrome steels, chrome-nickel and the like, containing at least 30 12 per cent chromium, comprising a mixture consisting of from  $\frac{1}{2}$  of 1 per cent to 10 per cent by volume of hydrofluoric acid, from 5 to 20 per cent by volume of chromic acid, from 1 to 10 per 35 cent by volume of sulphuric acid, and water.

STEPHEN F. URBAN.